

May 19, 1953

L. L. STOTT ET AL  
PRODUCTION OF STRIP STOCK FROM  
POLYHEXAMETHYLENE ADIPAMIDE

Filed Aug. 9, 1949

2,638,631

4 Sheets-Sheet 1



May 19, 1953

L. L. STOTT ET AL  
PRODUCTION OF STRIP STOCK FROM  
POLYHEXAMETHYLENE ADIPAMIDE

Filed Aug. 9, 1949

2,638,631

4 Sheets-Sheet 2

Fig. 2.



Fig. 3.



INVENTOR  
Louis L. Stott  
Paul L. Shurr  
BY  
Synnestvedt & Lechner  
ATTORNEYS

May 19, 1953

L. L. STOTT ET AL  
PRODUCTION OF STRIP STOCK FROM  
POLYHEXAMETHYLENE ADIPAMIDE

2,638,631

Filed Aug. 9, 1949

4 Sheets-Sheet 3

Fig. 4.



Fig. 5.



INVENTOR

Louis L. Stott  
Paul L. Shurr  
BY  
Stern, Lechner  
ATTORNEYS

May 19, 1953

Filed Aug. 9, 1949

**L. L. STOTT ET AL**  
**PRODUCTION OF STRIP STOCK FROM**  
**POLYHEXAMETHYLENE ADIPAMIDE**

2,638,631

4 Sheets-Sheet 4



Louis L. Stott INVENTOR  
Paul L. Shurr  
BY  
Symmes, Stott & Fischer  
ATTORNEYS

## UNITED STATES PATENT OFFICE

2,638,631

PRODUCTION OF STRIP STOCK FROM  
POLYHEXAMETHYLENE ADIPAMIDELouis L. Stott and Paul L. Shurr, Reading, Pa.,  
assignors to The Polymer Corporation, Reading,  
Pa., a corporation of Pennsylvania

Application August 9, 1949, Serial No. 109,336

1 Claim. (Cl. 18—55)

1

This invention relates to a method for forming strip stock from one of the high melting nylons, i. e., from polyhexamethylene adipamide.

The invention is concerned with that type of strip forming operation in which the molten nylon is continuously fed to the entrance nip of a pair of forming rolls, the formed strip being drawn from the rolls under tension. In this general type of operation certain special problems are encountered, particularly when forming relatively thin strip stock, for example strip stock less than .020 inch in thickness.

The invention relates to the establishment of certain operating temperatures for the molten nylon being fed to the rolls, and also to the drawing of the formed strip from the forming rolls under substantial tension in a direction in alignment with the plane of the pass between the rolls, such temperatures and drawing being correlated and arranged to enable production of sound strip stock even of quite thin gauge, for instance .008 inch in thickness.

Other objects of the invention include arrangement of the equipment to facilitate adjustment or regulation thereof so as to accommodate the equipment to the production of strip stock of different widths and thicknesses.

It is of importance in an operation of the character referred to above that the roll temperature be quite accurately maintained for a given condition of strip production, for instance with a given temperature and rate of feed of the molten nylon to the forming rolls, and with this in mind, the invention provides for accurate maintenance of roll temperature, by the circulation of a heat transfer medium through the rolls, as will further appear.

A further advantage of the capability of accurate regulation of roll temperature is that some of the properties of the formed strip may thereby be varied and accurately controlled at will. For instance, the tensile strength, elongation and rigidity may be controlled by regulation of the roll temperature.

Still other objects of the invention include provision for handling the polyamide in such manner as to minimize opportunity of the polyamide to oxidize in the molten condition, and to minimize tendency toward development of gas bubbles in the formed strip or development of surface markings thereon.

How the foregoing and other objects and advantages are attained will appear more fully from the following description referring to the accompanying drawings, in which—

2

Figure 1 is a longitudinal vertical sectional view through equipment arranged for carrying out the present invention:

Figure 2 is a transverse vertical section taken as indicated by the section line 2—2 on Figure 1;

Figure 3 is a horizontal view of certain portions of the equipment taken substantially as indicated by the line 3—3 on Figure 1, but with upper portions of the equipment removed;

Figure 4 is a longitudinal sectional view through the nozzle for delivering molten nylon to the forming rolls, the arrangement of this figure being shown on an enlarged scale;

Figure 5 is an enlarged detailed view of a portion of the nozzle shown in Figure 4;

Figure 6 is an axial sectional view through one of the forming rolls, this view being taken as indicated by the section line 6—6 on Figure 1, but being shown on an enlarged scale and also further showing connections for the circulation of a heat transfer medium through the roll;

Figure 7 is a plan view of the pair of forming rolls and of the connections for supplying a heat transfer medium thereto; and

Figure 8 is a sectional view of a detail taken as indicated by the line 8—8 on Figure 6.

The equipment illustrated in Figures 1 to 3, inclusive, comprises a vessel 7 adapted to contain a liquid cooling bath, the level of which appears at L in Figure 1. Liquid may be introduced into the vessel 7 through the inlet connection 8, which may advantageously be valved.

A frame 10 is mounted at the upper edge of the vessel 7 and serves as a support for the pair of forming rolls 11—12 which are fixed on shafts 13—14. The mounting of the rolls themselves, as illustrated herein conforms with that more fully disclosed and claimed in copending application of Robert C. Rahm, Serial No. 39,954, filed July 21, 1948, issued as U. S. Patent No. 2,627,085 on February 3, 1953, which application is assigned to the assignee of the present application. The adjustment and drive mechanism associated with the rolls also conforms with the disclosure of said copending application and since the present invention is not concerned with the arrangement of these parts per se, they need not be described in detail herein. Briefly, however, it is noted that the rolls are adapted to be driven from a power shaft 15 carrying gears 16—17 which mesh with gears 18—19 fixed on shafts 20—21, the latter shafts carrying worms, such as indicated at 22 and 23 which mesh with worm wheels such as shown in Figure 3 at 24 and 25, these worm wheels being fixed to the roll mount-

40  
45  
50  
55

ing shafts 13 and 14. The roll 11 is adjustable with relation to the roll 12, so as to vary the spacing between the rolls by means of an adjustable support for shaft 13 including traveling blocks 26 associated with manually adjustable screws 27.

According to the invention, a screw extruder is preferably employed for melting the polyamide being used and for feeding the molten polyamide to the entrance nip of the forming rolls. The details of construction of the extruder device itself need not be considered herein but it may be noted that this device has a hopper 30 adapted to receive the polyamide in granular form. The polyamide is fed from this hopper into the bore of the extruder proper indicated at 31, in which a screw advances the material toward the left when viewed as in Figure 1. The material is heated and melted by heater elements indicated in outline at 32 and is delivered in molten condition through the nozzle 33 which has its delivery opening close to the entrance nip between the rolls 11-12.

The formed strip is delivered downwardly substantially vertically from the rolls in a run such as shown at S'. This initial run of the strip from the forming rolls is defined by placement of a guide element, preferably a flanged roll 34 below the forming rolls 11-12. After passage around the guide element 34, the strip travels in a run S<sup>2</sup> upwardly at an incline, being drawn by the pairs of drawing rolls 35 and 36. After delivery from rolls 36, the strip material may be delivered to a trimmer or it may be wound up or otherwise packaged for shipment or the like.

The guide element 34 is mounted between the lower ends of a pair of generally upright supporting straps 37-31, the upper ends of these straps having slots 38 therein cooperating with supporting bolts 39 by means of which the straps are carried by supports 40 secured to the frame 10. The bolts 39 serve to adjustably fix the guide element 34 in any of a variety of positions including that shown in full lines in Figure 1 and also other positions, for instance as shown in dot-and-dash lines at 34a in Figure 1.

For purposes which will appear more fully hereinafter, a heating or cooling coil 41 may be positioned below the surface of the liquid in the cooling bath. This coil or other suitable means may be employed for temperature regulation, advantageously for cooling the liquid of the bath through which the strip is drawn after it is formed by the forming rolls.

It is preferred to employ a nozzle for the extruder of the type shown in Figures 4 and 5. The nozzle member 42 of this arrangement extends beyond the feeding screw of the screw extruder and is provided with a cavity 43 at its entrance end for receiving a screen pack for screening the molten nylon before entrance into the nozzle. The nozzle member 42 is surrounded by heater elements diagrammatically indicated at 44, and the delivery nozzle proper is associated with the delivery end of the member 42. This delivery nozzle comprises a pair of plates 45 and 46, the former comprising a flat plate and the latter having an aperture 47 for cooperation with the nozzle member 42 and further having a flaring delivery recess 48. As is shown, this recess flares so as to spread the molten nylon along the entrance nip between the rolls. In addition, the recess 48 is tapered transversely of the member 46 so that the delivery passage becomes progressively thinner as it

widens toward the delivery port. This configuration is of importance since it maintains the column of material being fed under pressure all the way to the point of discharge. This aids in minimizing formation of gas bubbles in the material. Indeed, in the construction of the entire nozzle, the several passages thereof are of progressively dimensioned cross-sectional flow area, so that somewhat of a back pressure is imposed on the material all the way back to the feeding screw in the extruder itself. Thereby the formation of gas or air bubbles within the material delivered from the extruder is greatly diminished.

It is of importance that the nozzle member 42 is maintained at a temperature above the freezing point of the polyamide and attention is also called to the fact that the heater diagrammatically indicated at 44 in Figure 4 extends all the way out to a point adjacent the nozzle tip, and this aids in maintaining even the nozzle tip at the desired high temperature.

The structure and arrangement of the forming rolls themselves is best illustrated in Figures 6, 7 and 8. As seen in Figure 6, roll 11 is provided with a hollow interior, being closed at one end by the closure member 49. At its other end the shaft 13 is also provided with an interior passage through which a tube 50 projects, with its inner end lying internally of the roll itself. Spaced discs 51 are arranged within the roll, each having an oversized central aperture accommodating the tube 50 and further having additional apertures as indicated at 52 for circulation of a heat transfer medium. Toward its left end when viewed as in Figure 6, the tube 50 is extended for connection with the flexible hose or the like 53. Another flexible hose 54 communicates with the annular passage 55 formed between the tube 50 and the inner wall of roll shaft 13, this latter connection being made through a fitting 56. Suitable internal rotative joints are provided to accommodate rotation of the roll 11 and its shaft 13, independently of the fluid supply and discharge connections 53, 54 and 56. Circulation of heat transfer medium is effected by introducing such medium through the flexible hose 53 from which it is delivered to the tube 50 and thence to the interior of the roll itself. The return circulation is effected through the ports 52 in the discs 51 and also in the annular space surrounding the tube 50, discharge being effected through the annular passage 55 and ultimately through the flexible hose 54.

Similar connections for circulation of heat transfer medium through roll 12 are provided, the flexible hose connections for this roll being indicated in Figure 7 at 57 and 58.

By virtue of the employment of the flexible hose connections, any required adjustments in relative positions of the rolls may be accommodated.

The heat transfer medium may be circulated through the rolls for the purpose of heating up the rolls prior to feed of molten nylon thereto; and during strip formation this heat transfer medium is employed for close regulation of the roll temperature, according to the particular conditions of operation. Such close regulation is advantageously achieved by employment of thermostatic control of heat transfer equipment through which the medium is passed after it is discharged from the rolls and before it is returned thereto. For most operations, especially where substantial quantities of molten material are be-

ing fed to the rolls, the heat transfer medium serves to carry heat away from the rolls.

The rolls 11 and 12 should desirably have a nicely polished or smooth surface and may be made of a variety of metals, including such metals as tool steel, stainless steel, etc. The pairs of drawing rolls 35 and 36 are advantageously made of rubber or some similar resilient compound having relatively high friction characteristics to provide for effective gripping and drawing of the formed strip. The drawing rolls should be driven at a rate somewhat faster than the rate of driving of the forming rolls 11-12, and the pressure of interengagement of the drawing rolls with the formed strip, and also the frictional characteristics of the drawing rolls should be such that considerable tension is provided.

The tension applied by the drawing rolls significantly affects the properties of the finished strip. Generally speaking, the fabrication of relatively thin strip, i. e., strip thinner than .020", requires greater tension than the fabrication of relatively thick strip, for example, strip whose thickness exceeds .050". The application of considerable tension during the fabrication of thin strip is important in producing strip substantially free of wrinkles, and also is of importance in avoiding the tendency for the formed strip to take a set with sharp curvature.

The effect of tension in overcoming the tendency to waviness is apparent in the following tables, in which are compared the characteristics of strip of several thicknesses, fabricated in separate runs in which the only variation in operating conditions was the tension applied to the strip. It should be emphasized that because of the difficulty of accurately measuring tension the individual figures are subject to some margin of error although the relative results for the various gauges are considered entirely representative of true conditions of operation.

Table 1

These examples illustrate the effect of varying the tension applied to the strip in the fabrication of material of .011" to .012" thick and 2 3/8" to 2 1/2" wide. The unit pressures were compiled on the basis of separate measurement of the cross sectional area for each run.

| Lbs. Tension | Lbs./Sq. Inch | Characteristics of Tape |
|--------------|---------------|-------------------------|
| 40           | 1,700         | Tape breaks.            |
| 23           | 900           | Normal tension.         |
| 12           | 460           | Somewhat wavy.          |
| 2            | 76            | Very wavy.              |

Table 2

These examples relate to the production of tape of .015" to .016" in thickness and 2 3/8" to 2 1/2" in width. Unit pressures in this and the following examples were calculated on the basis of a single measurement of cross sectional area for all runs.

| Lbs. Tension | Lbs./Sq. Inch | Characteristics of Tape |
|--------------|---------------|-------------------------|
| 150          | 3,900         | Tape breaks.            |
| 130          | 3,400         | Normal tension.         |
| 22           | 560           | Somewhat wavy.          |
| 2            | 57            | Very wavy.              |

Table 3

These examples illustrate the effect of varying tension on tape .018" to .019" in thickness and 2 3/8" to 2 1/2" wide.

| Lbs. Tension | Lbs./Sq. Inch | Characteristics of Tape |
|--------------|---------------|-------------------------|
| 140          | 3,300         | Tape breaks.            |
| 106          | 2,500         | Normal tension.         |
| 89           | 2,100         | Somewhat wavy.          |

Table 4

These examples are illustrative of the very much lower tensions employed in accordance with the invention in fabricating strip which is very much thicker than the strip of the preceding examples, the strip of this example being .060" to .062" in thickness, and from 2 3/4" to 2 7/8" in width.

| Lbs. Tension | Lbs./Sq. Inch | Characteristics of Tape |
|--------------|---------------|-------------------------|
| 25           | 127           | Tape breaks.            |
| 21           | 97            | Normal tension.         |

It will be seen from the data set forth above that when working with thin strip the range for producing tape which is free from waviness is upwards of 150 lbs./sq. in. and preferably upwards of 450 lbs./sq. in., the upper limit of tension being established by the point at which the strip breaks. It should be pointed out in connection with the upper limit that in the examples above set forth, the apparatus was operated with the water level in the bath illustrated in Figure 1 somewhat higher than that illustrated in the figure, that is to say, the experimental data was obtained when the bath level was almost touching the lower portion of the rolls for the strip below .020" thickness, and in contact with the rolls on the .060" to .062" material. We have found that as the water level is lowered it becomes increasingly more difficult to break the tape. In particular, we have found that when the level of the bath is at least two inches below the point where the tape leaves the forming rolls, the .018" tape (the subject matter of Table 3) cannot be broken at all, but rather undergoes elongation, with corresponding orientation of the molecules.

The liquid bath in the vessel 1 serves to bring down the temperature of the formed strip, so that it may readily be handled as it is delivered from the equipment. In some cases the level of the liquid cooling bath may be somewhat higher than indicated in Figure 1 and may be sufficiently high to contact the lower portions of the rolls, although for accuracy of temperature regulation of the rolls, it is preferred to avoid contact of the liquid with the rolls.

Water may be employed as the cooling liquid in the bath and it is contemplated to employ some rust preventive or inhibitor therein, especially in the event of contact of the bath with the rolls, a particularly effective inhibitor being potassium bichromate, which serves the purpose but at the same time is not subject to being carried out of the bath on the formed strip. In the event that the bath level is kept high enough to contact the rolls it is contemplated that the rolls be equipped with wipers to remove water therefrom, for instance wipers of the character disclosed in the copending application of Montross and Schurr,

7  
Serial No. 38,966, filed July 16, 1948, issued as Patent No. 2,624,913 on January 13, 1953, which application is assigned to the assignee of the present application.

When making thin strip we have found that this tendency for the strip to coil up sharply is also influenced by the position of the guide element 34 and can be greatly diminished when the guide element is positioned substantially below the forming rolls, i. e., so that the initial run of the strip being drawn from the forming rolls extends in a path substantially in alignment with the pass between the rolls. A position such as indicated in full lines in Figure 1 is desirable when making very thin strip, although the position may be shifted somewhat, for instance to the position indicated in dotted lines at 34a, depending upon the thickness of the strip being formed.

Still another important factor in producing thin strip of good quality and especially thin strip having a minimum of transverse ridges or wrinkles is the temperature of the forming rolls. According to the invention, when making relatively thin strip, for instance less than .015" in thickness, the temperature of the forming rolls should be quite accurately controlled within temperature ranges as given herebelow.

To consider an example of preferred temperature conditions, reference is made to a typical operation, producing strip from polyhexamethylene adipamide, which has a melting point of about 507° F. and a somewhat lower freezing point at about 473° F. When forming strip from this polyamide, it is preferred to deliver the molten polyamide to the entrance nip of the forming rolls at a temperature somewhat above the freezing point, but preferably not substantially above the melting temperature, an effective range being from 480° F. to 515° F. Somewhat higher temperatures may be used, for instance up to about 550° F., but excessively high temperatures are to be avoided because of the tendency for the material to form bubbles and to oxidize. Moreover, excessively high temperatures interfere with the desired solidification of the material as it passes through the rolls.

It should be borne in mind that the temperature of the rolls is dependent not only on the temperature of the roll control liquid but also on the volume and temperature of the molten nylon being fed to the entrance nip of the rolls. In any case, the conditions should be adjusted so as to maintain a roll temperature above about 180° F. but below about 350° F. when making thin strip from polyhexamethylene adipamide. The temperature is most desirably kept above 200° F., a particularly effective range being between 220° F. and 300° F.

In regulating the feed of the molten material, the screw extruder 31 and the speed of the rolls 11 and 12 should be operated at such rate as to maintain a slight excess or reservoir of the

molten nylon in the entrance nip of the forming rolls.

With respect to the reference herein to formation of strip stock, it should be understood that the invention is not only applicable to the production of plain flat strip but also to strip of shaped section, for instance beaded material or the like, in which event the forming rolls would be appropriately shaped to give the desired strip section.

15 In practicing the invention it is of importance that the polyamide used be of very low moisture content prior to melting, preferably below .25% water content by weight. Therefore, we prefer to preliminarily and carefully dry the granular or flake material before melting, and this is especially important in the case of polyhexamethylene adipamide, which is preferably carefully vacuum dried. In the absence of such drying an excess of bubbles forms in the material and the formed strip has lower elongation and has a tendency to brittleness.

20 Strip formed in accordance with the present invention is substantially free of bubbles and other defects either within the piece or on the surface thereof. The edges of the strip are frequently somewhat irregular in view of which trimming is contemplated. The formed strip itself has excellent physical characteristics, including toughness, and high tensile strength.

25 In the case of a strip of .010 in thickness, made with rolls at a temperature of about 220° F., the tensile strength was 9540 lbs./sq. in., and the elongation 194% in a 2 in. gauge length.

30 The techniques covered by this invention are applicable to polyhexamethylene adipamide with or without fillers such as graphite, coloring ingredients, antioxidants, or other additions.

We claim:

40 40 The method for forming substantially wave-free strip stock of thickness less than .020" from polyhexamethylene adipamide, which method comprises feeding molten polyamide to the entrance nip of a pair of forming rolls maintained at a temperature of from 180° F. to 350° F., and drawing the formed strip from the forming rolls under a tension of more than 150 lbs./sq. in., but less than that which would break the strip or appreciably orient the polyamide.

50 LOUIS L. STOTT.  
PAUL L. SHURR.

References Cited in the file of this patent

UNITED STATES PATENTS

| Number    | Name    | Date           |
|-----------|---------|----------------|
| 2,048,686 | Conklin | July 28, 1936  |
| 2,212,772 | Graves  | Aug. 27, 1940  |
| 2,244,208 | Miles   | June 3, 1941   |
| 2,289,774 | Graves  | July 14, 1942  |
| 2,295,942 | Fields  | Sept. 15, 1942 |
| 2,336,159 | Bent    | Dec. 7, 1943   |